

## UNITED STATES PATENT OFFICE

2,691,578

## IRON-MOLYBDENUM TITANIUM BASE ALLOYS

Schuyler A. Herres and Thomas K. Redden, Las Vegas, Nev., assignors to Allegheny Ludlum Steel Corporation, Brackenridge, Pa., a corporation of Pennsylvania

No Drawing. Application April 12, 1951,  
Serial No. 220,722

7 Claims. (Cl. 75—177)

1

This invention relates to new and improved titanium-base alloys containing iron and molybdenum and a hardening element of the type of oxygen and nitrogen. These alloys are suitable for more critical utilizations requiring an improved tensile and yield strength, a good ductility for cold working, an excellent corrosion resistance and which may be reversibly hardened and softened by heat treatment. This application is a continuation-in-part of our application, Serial No. 118,723, entitled "Titanium Alloys," filed September 29, 1949.

Alloys of the type with which we are here concerned are suitable for structural uses where higher strength and lighter weight are essential such as in aircraft and turbine utilizations.

An object of our invention has been to provide new and improved titanium-base alloys containing iron and molybdenum metal alloying elements and gaseous alloying elements of the class of nitrogen and oxygen.

The constituents of these alloys fall within the following critical ranges:

TABLE I

25

A

O<sub>2</sub>=0.02 to 0.40%

Fe=0.5 to 3.0%

Mo=1.0 to 5.0%

B

N<sub>2</sub>=0.05 to 0.25%

Fe=0.5 to 3.0%

Mo=1.0 to 5.0%

C

O<sub>2</sub>=0.02 to 0.40%N<sub>2</sub>=0.02 to 0.30%

Fe=0.5 to 3.0%

Mo=1.0 to 5.0%

Balance titanium in each of A, B and C.

For optimum results in alloy A, the iron should be a minimum of about 25 times the oxygen content and not substantially less than about  $\frac{1}{2}$  of the molybdenum content. The oxygen is used within the permissible range and is proportioned to the molybdenum and iron to provide hardening without excessive hardness.

For optimum results in alloy B, the iron should be a minimum of about 10 times the nitrogen content and not substantially less than about  $\frac{1}{2}$  of the molybdenum content. The nitrogen is used within the permissible range and is proportioned to the molybdenum and iron to provide hardness without excessive hardness.

In alloy C where both nitrogen and oxygen are used, their ranges are substantially the same, except that the range of nitrogen is slightly greater than where it is used separately, as in alloy B.

The lower and upper limits of the iron and molybdenum are the same as before and the ratios are substantially the same.

The following table sets forth alloys within the ranges of Table I, giving tensile properties and hardness for representative optimum alloys:

TABLE II

Titanium-base alloys containing iron and molybdenum and oxygen or nitrogen

| Composition (Balance Ti) |                |     |     | Tensile Strength | Percent Elong. | R. A., Percent | BHN |
|--------------------------|----------------|-----|-----|------------------|----------------|----------------|-----|
| O <sub>2</sub>           | N <sub>2</sub> | Fe  | Mo  |                  |                |                |     |
| 0.10                     | —              | 0.8 | 1.2 | 90,000           | 24             | 26             | 197 |
| 0.10                     | —              | 1.2 | 1.8 | 96,000           | 23             | 54             | 201 |
| 0.10                     | —              | 1.6 | 2.4 | 102,200          | 23             | 52             | 217 |
| 0.10                     | —              | 2.0 | 3.0 | 118,200          | 21             | 46             | 248 |
| 0.1                      | —              | 3.0 | 4.5 | 150,000          | 21             | 37             | 311 |
| 0.2                      | —              | 1.6 | 2.4 | 113,200          | 21             | 56             | 255 |
| —                        | 0.12           | 1.6 | 2.4 | 132,200          | 22             | 36             | 269 |
| 0.35                     | —              | 2.0 | 3.0 | 157,000          | 11             | 17             | —   |
| 0.40                     | —              | 1.0 | 1.5 | 146,000          | 22             | 44             | —   |
| 0.35                     | —              | 1.6 | 2.4 | 143,000          | 18             | 53             | —   |
| —                        | 0.27           | 1.6 | 2.4 | 162,100          | 19             | 48             | —   |
| —                        | 0.12           | 2.0 | 3.0 | 152,000          | 20             | 58             | —   |
| —                        | 0.25           | 2.0 | 3.0 | 171,000          | 19             | 48             | —   |
| —                        | 0.25           | 1.7 | 3.0 | 204,000          | 7              | —              | 405 |

The alloys set forth in the Table II were made by tungsten-arc melting in a water cooled copper crucible under an argon atmosphere. These alloys were subjected to the normal heat treatment hereinafter set forth, followed by air cooling. That is, they were hot worked at about 1400° to 1700° F., annealed at about 1300° F., and then air cooled. The following sets forth typical quench hardening characteristics of these alloys, as indicated by a representative alloy:

TABLE III

Quench hardening

40 A. Composition:

|                  |      |
|------------------|------|
| O <sub>2</sub> — | 0.25 |
| N <sub>2</sub> — | —    |
| Fe—              | 1.6  |
| Mo—              | 2.4  |
| Balance titanium | —    |

| Quenching Temperature | Vickers Hardness A |
|-----------------------|--------------------|
| 1,400° F.             | 360                |
| 1,500° F.             | 451                |
| 1,600° F.             | 540                |
| 1,700° F.             | 499                |

Samples were quenched in cold water from the above temperatures.

These alloys are capable of being hardened by rapid cooling from above about 1300° F. After hardening, they may be softened by holding at temperatures below 1300° F. and slow cooling.

## 3

The normal heat treatment involves hot working them within an optimum range of about 1400° to 1700° F. and annealing at about 1300° F. after working. Generally speaking, hot working within a temperature range of about 1400° to 1800° F., followed by cooling in air produces desirable properties for most structural uses. A subsequent anneal or stress relief (solution treatment) is preferred to obtain uniformity of properties. This is accomplished by reheating to a temperature within the range of about 1200° to 1600° F. and cooling at a suitable rate. Alloys B and C respond favorably to heat treatment and may be hardened by rapid cooling, as water quenching from temperatures above about 1500° F., or 15 softened by relatively slow cooling from the same temperature.

Ferro-molybdenum is used in making these alloys (may be composed of about 60% molybdenum and 40% iron) to carry out the novel 20 procedure set forth in our copending application Serial No. 118,723, above mentioned.

All the alloys may also be hardened by an age 25 hardening treatment on holding at temperatures within a range of 400° to 1000° F. for a length of time depending upon the temperature employed, see Tables IV and V.

TABLE IV

| Composition (Balance Ti) |     |     | Heat Treatment      | Tensile Strength | Percent Elong. | Percent R. A. |
|--------------------------|-----|-----|---------------------|------------------|----------------|---------------|
| O <sub>2</sub>           | Fe  | Mo  |                     |                  |                |               |
| 0.1                      | 3.0 | 4.5 | 143 hrs. at 600° F. | 178,100          | 9              | 11            |
| 0.1                      | 3.0 | 4.5 | 1,300° F., 1 hr.    | 142,800          | 15             | 31            |
| .25                      | 1.6 | 2.4 | 143 hrs. at 600° F. | 165,100          | 5              | 16            |
| .25                      | 1.6 | 2.4 | 1,300° F., 1 hr.    | 143,000          | 18             | 53            |
| .2                       | 2   | 3   | 1,300° F., 1 hr.    | 158,800          | 13             | 45            |
| .2                       | 2   | 3   | 300 hrs. at 600° F. | 173,600          | 6              | 17            |

TABLE V

## Composition:

|                | Percent |
|----------------|---------|
| O <sub>2</sub> | 0.1     |
| Mo             | 2.4     |
| Fe             | 1.6     |

Rockwell "A" hardness after heat treatment  
samples quenched from 1300° F. in water and  
given following treatment

| Hours..... | 400° F. |      |    | 600° F. |      |    | 800° F. |      |      | 1,000° F. |      |    | 1,200° F. |      |      |
|------------|---------|------|----|---------|------|----|---------|------|------|-----------|------|----|-----------|------|------|
|            | 2       | 16   | 50 | 2       | 16   | 50 | 2       | 16   | 50   | 2         | 16   | 50 | 2         | 16   | 50   |
|            | 62      | 63.5 | 61 | 65.5    | 63.5 | 65 | 66      | 62.5 | 62.5 | 59        | 58.5 | 60 | 59.5      | 60.5 | 60.5 |

All the alloys are also capable of being hardened, following rapid cooling from a temperature above about 1200° F., by an aging and precipitation hardening mechanism on reheating and holding for various periods within a temperature range of about 700° to 1200° F. The time of holding is less, the higher the aging temperature in this range and the effect is reversible, so that the alloy may again be softened by reheating to a high temperature. The alloys may also be hardened by cold working, i. e., mechanical reduction in cross-sectional area at temperatures below about 1200° F., and may be softened again by heating to a temperature above about 1200° F. and slowly cooling. The temperature and the time employed in the softening operation will

depend upon the degree of cold work accomplished.

All the alloys may be surface hardened by heating in air or atmospheres, mixtures, or fused baths that provide nitrogen or oxygen or both for combination with the titanium. For example, titanium heated in the presence of oxygen for about one hour at 1900° F. is hardened for a depth of about .050 of an inch below the surface with a maximum surface hardness of 400 Brinell. Similar surface hardening effects are produced by heating titanium or the alloys in a nitrogen-rich atmosphere, such as ammonia gas at temperatures as low as 950° F. The depth and degree of hardness produced is controlled by time and temperature of exposure as well as the composition of the atmosphere or bath used.

In accordance with our procedure, ferrous metal, and particularly a ferrous combination of molybdenum, is added to the titanium while it is in a molten state and an ambient atmosphere is maintained that is non-contaminating of the titanium. The oxygen or nitrogen may be added in controlled amounts by introduction of the gas or gases to the furnace during melting or by additions as compounds of oxygen or nitrogen with titanium.

What we claim is:

1. A titanium-base alloy consisting of .10 to 30 .40% oxygen, about .8 to 3% iron, about 1.2 to 4.5% molybdenum, and the remainder titanium.

2. A titanium-base alloy consisting of .12 to 25 .27% nitrogen, about 1.6 to 2% iron, about 2.4 to 3% molybdenum, and the remainder titanium.

3. A titanium-base alloy consisting essentially of at least one alloying gas within the range specified of: .02 to .40% oxygen and .05 to .25% nitrogen, about .5 to 3% iron, about 1 to 5% molybdenum, and the remainder titanium; the 40 alloy being characterized by its improved tensile and yield strengths with adequate ductility, corrosion resistance, and ability to be reversibly hardened and softened by temperature treatment.

4. A titanium-base alloy as defined in claim 3 45 wherein the iron content is a minimum of about 25 times its oxygen content and a minimum of

about 10 times its nitrogen content and is not substantially less than about one-half of the molybdenum content.

5. A titanium-base alloy consisting of .02 to 65 .40% oxygen, about .5 to 3% iron, about 1 to 5% molybdenum, and the remainder titanium; the iron content being a minimum of about 25 times the oxygen content and being not substantially less than one-half of the molybdenum content.

6. A titanium-base alloy consisting of .05 to 70 .25% nitrogen, about .5 to 3% iron, about 1 to 5% molybdenum, and the remainder titanium; the iron content being a minimum of about 10 times the nitrogen content and not substantially less than about one-half of the molybdenum content.

## 5

7. A titanium-base alloy consisting essentially of .02 to .40% oxygen, .02 to 30% nitrogen, about .5 to 3% iron, about 1 to 5% molybdenum, and the remainder titanium; the alloy being characterized by its improved tensile and yield strengths with adequate ductility, corrosion resistance, and the ability to be reversibly hardened and softened by temperature treatment.

References Cited in the file of this patent

## UNITED STATES PATENTS

| Number    | Name         | Date          |
|-----------|--------------|---------------|
| 2,188,765 | Young        | Jan. 30, 1940 |
| 2,258,992 | Mansfield    | Oct. 14, 1941 |
| 2,294,648 | Ansel et al. | Sept. 1, 1942 |
| 2,467,367 | Austin       | Apr. 19, 1949 |

## 6

| Number      | Name           | Date          |
|-------------|----------------|---------------|
| 2,497,667   | Gresham et al. | Feb. 14, 1950 |
| 2,520,753   | Ball et al.    | Aug. 29, 1950 |
| 2,554,031   | Jaffee et al.  | May 22, 1951  |
| 5 2,575,962 | Jaffee et al.  | Nov. 20, 1951 |
| 2,588,007   | Jaffee         | Mar. 4, 1952  |

## FOREIGN PATENTS

| Number     | Country | Date          |
|------------|---------|---------------|
| 10 718,822 | Germany | Mar. 24, 1942 |

## OTHER REFERENCES

AF Technical Report No. 6218, Part 2, "Research and Development on Ti Alloys," published 1950 by Battelle Memorial Institute, page 66.  
Metallurgia, June 1949, page 72.